

## 1

3,484,289

### METHOD OF PROCESSING METALS FOR USE IN ALLOYING FURNACES

Alvin Wasserman, Detroit, Mich.

(1521 Charrington, Birmingham, Mich. 48010)  
No Drawing. Filed Nov. 3, 1965, Ser. No. 506,274

Int. Cl. B08b 5/00

U.S. Cl. 134—26

6 Claims

#### ABSTRACT OF THE DISCLOSURE

A scrap recovery method in which "unused" scrap metal of odd-shapes but known metallurgical composition is pre-shaped and pre-treated in such fashion as to render them suitable for use as a constituent in quality alloy melting furnaces by first cutting said "unused" scrap metal into parts of appropriate size, secondly, chemically cleaning the cut parts and thirdly, heat treating the cut and cleaned parts to condition them for shipment to the steel making plants.

This invention relates to a method of processing metal sheets so as to make them useful as constituents, along with other metals, in melting furnaces which produce alloys; and more particularly to a method of sizing and cleaning metals of known metallurgical composition to provide elements useful for such alloying furnaces.

Scrap steel which results from metal working processes is often of the proper metallurgy but improper physical configuration for use in other metal working operations, and is normally bailed and delivered to steel mills for use as a constituent in the production of "new" steel in blast furnaces. As such, it has a value not appreciably higher than "used" scrap which derives from the salvaging of obsolete or inoperative devices such as automobiles, which have a large steel content. This metal working scrap, at least in certain forms, such as sheets or slugs, would have a much greater value if it could be employed in melting furnaces for the production of quality alloys. Use in this manner is normally prevented by the odd physical configuration of the material which makes it unsuitable for both shipment and use in melting furnaces having relatively small apertures and the contamination of the material by dirt and oxides.

It is therefore a broad object of the present invention to provide a process for operating upon scrap material from metal working operations, and sheet and plate scrap material in particular, in order to render it useful as an input to alloying furnaces.

The scraps so processed must be of a known and uniform metallurgy. Scrap steel having a low carbon content has a particularly high economic value as it may be used as a base in making special alloy steels in competition with low carbon steel sheet or plate produced by a mill and sold directly for this purpose.

As disclosed in the following description of a preferred embodiment of my inventive process, the scrap sheet or plate is first formed into segments of a relatively uniform size, all having dimensions equal to or less than a maximum. In the preferred embodiment this is done by feeding sheets of the material into stamping presses which die cut the sheets into relatively small shapes, such as squares. The odd shape of the scrap part will often prevent the formation of segments having the shape of the dies, but the segments formed will be no larger than the full die cut segments. These sized segments are collected and delivered, preferably by automatic means, to a processing device which first washes the segments by tumbling them through streams of detergent solutions and then dries the clean segments by subjecting them to a relatively high

## 2

temperature for a sufficient time to completely evaporate the cleaning solution and any other surface moisture. This final heat processing allows the cleaned segments to be bailed and shipped without any special protective coating as the newly cleaned surfaces are free of both oxide and oxide producing moisture.

It is therefore seen to be a preferred embodiment of the present invention to provide a process for operating on scrap from metal working operations to bring it into form and condition suitable for use in alloy melting furnaces which consists of the combination of first cutting the scrap into segments all having maximum outer dimensions; then washing the segments by tumbling them through detergent solutions, and finally subjecting the segments, immediately upon their removal from the washing apparatus, to an elevated temperature for a sufficient length of time to remove all moisture from their surface.

The "sterilized" segments formed by the above process provide the user of the melting furnace with a constituent which decreases the inclusions in the output of the furnace, produces less slag and results in a longer refractory life. The product is, therefore, directly competitive with alloying steels as produced directly by a mill.

Other objects, advantages and applications of the present invention will be made apparent by the following detailed description of a preferred embodiment of the process.

The preferred embodiment of the process is capable of operating upon metals of various configuration or metallurgy. A typical material will be sheets of a steel such as SAE 1010 which has a carbon content of less than 10%.

The sheets or plates are then fed to a stamping press which employs a die that preferably cuts a two inch by two inch square configuration. The irregularly shaped workpiece may be manually fed into the die so that a number of small, square segments are formed. On the edges of the sheet, the dies may not cut full squares, but all of the part cut by the die will have dimensions no larger than those of the die.

The segments thus formed are delivered to a washer where they are tumbled through jets or streams of a suitable liquid detergent of a high alkaline type commonly used for cleaning impurities from the surfaces of metals. The exact configuration of the washer and the length of time to which the segments are exposed to the detergent stream is dependent upon the particular configuration of the washer and the degree to which the particular scrap being processed is contaminated by dirt and oxides.

Immediately upon the removal of the washed segments from the washing process, they are subjected to a blast of 450 F. degree air for a period of two minutes. We have determined that if the air blast has a temperature of less than 300 F. degrees there is a tendency of thin oxide coating to form on the newly washed segments before the moisture is fully evaporated and/or vaporized. The atmosphere is continuously and rapidly ventilated during this time to remove all moisture. It has been found that this removes all surface moisture so that the segments will not begin to oxidize unless later subjected to moisture or a moist atmosphere.

Following this treatment, the segments are in condition for use in alloying furnace. The small maximum dimensions of the segments allow them to be employed in furnaces with small apertures and to easily intermingle with the other components in the melt.

It should be understood that any variety of available apparatus may be employed for stamping the segments and for washing and heating them.

Having thus described my invention, I claim:

1. The process for converting irregular steel sheets into a condition suitable for use as elements in an alloying

furnace comprising: forming the sheets into a plurality of small segments having a predetermined maximum dimension; washing the formed segments in a detergent solution; and, subjecting the washed segments, immediately upon removal from the washing process, to an air blast at an elevated temperature of not less than 300° F., in a ventilated atmosphere, for a sufficient time to vaporize all moisture on the surface of the segments and thereby prevent the formation of thin oxide coatings on the newly washed segments.

2. The process of claim 1 wherein the segments are washed by tumbling them through streams of a detergent solution.

3. The process of claim 1 wherein the segments are subjected to the temperature of at least 300 degrees F. for a period of at least two minutes.

4. In the process defined in claim 1, said blast of hot air comprising an air blast having a temperature of between 300° and 450° F.

5. The process as defined in claim 1, in which said

cleaning step comprises washing said segment in an aqueous detergent solution.

6. In the process defined in claim 5 said detergent solution being an alkaline solution.

#### References Cited

##### UNITED STATES PATENTS

|           |         |           |       |        |    |
|-----------|---------|-----------|-------|--------|----|
| 1,580,723 | 4/1926  | Hapgood   | ----- | 134—25 | XR |
| 2,356,807 | 8/1944  | Wulff     | ----- | 134—2  | XR |
| 2,714,574 | 8/1955  | Kearney   | ----- | 134—25 | XR |
| 2,977,255 | 3/1961  | Lowry     | ----- | 134—25 | XR |
| 3,163,929 | 1/1965  | Goodstein | ----- | 134—2  | XR |
| 3,346,417 | 10/1967 | Ehrlich   | ----- | 134—25 | XR |

10 MORRIS O. WOLK, Primary Examiner

J. T. ZATAROGA, Assistant Examiner

U.S. Cl. X.R.

15 20 75—129; 134—25, 29, 30, 37